

S. I. Potter.

## *Flagot for Railroad Rails.*

N° 61,565.

Patented Jan. 29, 1867.



Witnesses

Geo. W. Rothwell  
Solon C. Kamm

## Inventor

S. L. Potter  
Prof. Knight, Supy  
Mammals, atty

# United States Patent Office.

SAMUEL L. POTTER, OF WYANDOTTE, MICHIGAN.

*Letters Patent No. 61,565, dated January 29, 1867.*

## IMPROVED FAGGOT FOR RAILROAD RAILS.

The Schedule referred to in these Letters Patent and making part of the same.

TO ALL WHOM IT MAY CONCERN:

Be it known that I, SAMUEL L. POTTER, of Wyandotte, in the county of Wayne, and State of Michigan, have invented a new and improved Rail Pile; and I do hereby declare that the following is a full, clear, and exact description thereof, which will enable those skilled in the art to make and use the same, reference being had to the accompanying drawings, forming part of this specification, in which—

Figure 1 represents a transverse section of my improved pile or faggot, one half the actual size.

Figure 2 is a transverse section of the same, illustrating a manner of applying old railroad bars in place of the inner or intermediate iron bars of the pile.

Figure 3 represents a transverse section of the complete rail, full size.

Similar letters of reference indicate corresponding parts.

The subject of this invention is a peculiar arrangement of iron bars, in connection with a steel head of T form, the bottom of which steel head will be protected from undue heating, and the whole being adapted to be effectually welded together in the operation of rolling.

In fig. 1, a pile is shown, composed of three flat iron bars, *b*, of equal dimensions, (seven by one and a quarter inches,) placed one on the top of the other, and four narrower bars, *a*, two and a half by one inch, placed on the top bar *b*, the outer edges of the bars *a* being placed flush with the outer edges of the bars *b*, so that a space will be allowed between them to receive the lower part *c'* of a T-shaped steel bar; *c c'*, said part *c'* being two inches square in its transverse section, and the upper part *c* seven inches in width and one and three-quarters inch in thickness, the part *c* extending the whole width of the pile. This pile, when rolled, will produce a rail as shown in fig. 3, *A* being the steel head and *B* the iron neck and base. By this means it will be seen that the steel will be brought to a welding heat, and fully protected by the iron, as the steel will weld at a much lower heat than the iron, and the two metals will, during the process of rolling, be perfectly welded together.

Having thus described my invention, what I claim as new therein, and desire to secure by Letters Patent, is—

A pile or faggot for railroad bars, constituted of iron and steel bars, arranged substantially as herein represented and described.

To the above specification of my improved rail pile I have signed my hand this 8th of November, 1866.

SAMUEL L. POTTER.

Witnesses:

SOLON C. KEMON,  
GEO. W. ROTHWELL.